

# UNITED STATES PATENT OFFICE.

HENRI SCHMID, OF MÜLHAUSEN, GERMANY, ASSIGNOR TO BADISCHE ANILIN & SODA FABRIK, OF LUDWIGSHAFEN-ON-THE-RHINE, GERMANY, A CORPORATION.

## PROCESS OF PRODUCING BROWN SHADES ON FIBER.

1,092,542.

Specification of Letters Patent.

Patented Apr. 7, 1914.

No Drawing.

Application filed December 8, 1912. Serial No. 734,654.

To all whom it may concern:

Be it known that I, HENRI SCHMID, citizen of the Swiss Republic, residing at Mülhausen, Germany, have invented new and useful Improvements in Processes of Producing Brown Shades on Fiber, of which the following is a specification.

I have found that valuable and fast brown shades can be obtained on fiber in a simple manner by the oxidation, by means of a chlorate, of ortho-dianisidin dissolved in acid. In order to avoid damaging the fiber, it is preferred to use a solution of ortho-dianisidin in an organic acid, or in a mixture of an organic acid with a comparatively small quantity of mineral acid, for instance a quantity of mineral acid can be used which would only suffice to combine completely with one-fourth the quantity of base employed.

The use of a vanadium salt to assist in the reaction, as is usual in the production of anilin black, is not suitable for the purposes of my invention, because the vanadium salts act too energetically and cause a too rapid oxidation both of the bath and of the material which has been padded, so that, on steaming the material, only a light brown shade is obtained instead of a full dark brown shade. It is, however, often advisable to promote the reaction by means of suitable catalysts, as then the ortho-dianisidin is used up to the greatest advantage and a quick and certain action is insured. As instances of such catalysts, I mention metallic salts which react less energetically than vanadium salts and in particular iron salts and copper salts. As a rule, as small quantities as possible of these salts should be employed so as to prevent oxidation taking place too soon.

When preparing the padding or printing mixtures, the additions usual in such operations, such for instance as acetin, can be made. Also potassium ferrocyanid can be added and the peculiar effect is obtained that the shade varies according to the quantity of potassium ferrocyanid employed; for example, by suitable variation of the quantity employed, very bright and light orange to red-brown shades of excellent fastness can be obtained, or bright yellow-brown, orange-brown, or old gold, or rusty brown, or chamois, shades can be produced. In consequence of this action of the ferrocyanid, pat-

terns can be obtained by printing pastes containing potassium ferrocyanid on material which is already padded with the dianisidin mixture and then steaming the goods. Other variations can be obtained by printing a chlorate mixture, which may be of the usual kind generally employed for discharging coloring matters from fiber, on material which has already been developed either with or without white reserve effects. On steaming the material thus printed, beautiful golden yellow patterns on a brown ground are obtained. Dianisidin can be thus employed for the production of a very great number of different shades, such as hitherto could not be obtained by the oxidation of one and the same amin. In the case of all the shades obtained in the aforesaid manner, the material can be reserved either white or in colors by treating, with a reducing agent, the padded or printed material before steaming.

The following example will serve to illustrate further the nature of my invention, which, however, is not confined to this example. The parts are by weight: Prepare a padding liquor in the following manner: Dissolve 28 parts of ortho-dianisidin in 7 parts of 30% hydrochloric acid and from 18 to 20 parts of 90% formic acid and a little water, while warming. When the solution is cold, add a solution of 25 parts of sodium chloride dissolved in a little water and make up the whole with water to 1,000 parts. As a catalyst from 0.5 to 0.75 part of ferrous sulfate or potassium ferrocyanid can be added. Pad the material with this solution, dry, and steam in a Mather-Platt apparatus. A manganese bronze shade is thus obtained. If from 10 to 30 parts of potassium ferrocyanid be added to the padding bath, a brighter brownish orange shade is produced.

To produce a printing paste, the usual or any suitable thickenings and other suitable agents can be added.

Now what I claim is:

1. The process of producing brown shades on fiber by applying to the material ortho-dianisidin and less than one equivalent of mineral acid for each equivalent of ortho-dianisidin employed and a chlorate, and then causing the oxidation of the ortho-dianisidin substantially as hereinbefore described.

2. The process of producing brown shades on fiber by applying to the material ortho-

dianisidin and less than one equivalent of mineral acid for each equivalent of ortho-dianisidin employed and a chlorate and a suitable catalyzer, and then causing the oxidation of the ortho-dianisidin substantially as hereinbefore described.

3. The process of producing brown shades on fiber by applying to the material ortho-dianisidin and less than one equivalent of mineral acid for each equivalent of ortho-dianisidin employed and a chlorate and a small quantity of potassium ferrocyanid, and then causing the oxidation of the ortho-dianisidin substantially as hereinbefore described.

4. The process of producing brown shades on fiber by applying to the material ortho-dianisidin, an organic acid, a quantity of inorganic acid sufficient to combine with about one-fourth of the quantity of base employed, and alkali metal chlorate, and then causing the oxidation of the ortho-dianisidin.

5. The process of producing brown shades on fiber by applying to the material ortho-dianisidin and less than one equivalent of mineral acid for each equivalent of ortho-dianisidin employed and a chlorate, and then subjecting the material to the action of steam.

30 6. The process of producing brown shades

on fiber by applying to the material ortho-dianisidin and less than one equivalent of mineral acid for each equivalent of ortho-dianisidin employed and a chlorate and a suitable catalyzer, and then subjecting the material to the action of steam.

7. The process of producing brown shades with reserve effects on fiber by applying to the material ortho-dianisidin and less than one equivalent of mineral acid for each equivalent of ortho-dianisidin employed, and a chlorate, and then treating the material with a reducing agent and subjecting it to the action of steam.

8. The process of producing brown shades with reserve effects on fiber by applying to the material ortho-dianisidin and less than one equivalent of mineral acid for each equivalent of ortho-dianisidin employed and a chlorate and a suitable catalyzer, and then treating the material with a reducing agent and subjecting it to the action of steam.

In testimony whereof I have hereunto set my hand in the presence of two subscribing witnesses.

HENRI SCHMID.

Witnesses:

GEO. GIFFORD,  
ARNOLD ZUBER.